

## UNITED STATES PATENT OFFICE.

ALFRED OBERLE, OF CHICAGO, ILLINOIS, ASSIGNOR TO UNIVERSAL OIL PRODUCTS COMPANY, OF CHICAGO, ILLINOIS, A CORPORATION OF SOUTH DAKOTA.

## CARBONACEOUS FUEL AND PROCESS OF MAKING SAME.

No Drawing. Application filed May 9, 1923, Serial No. 337,878. Renewed January 13, 1928.

This invention relates to improvements in carbonaceous fuel, and a process of making the same, and refers more particularly to a fuel made from the carbon deposited in connection with the treatment of hydrocarbon oils, and particularly the carbonaceous substance separated from the oil during the cracking or destructive distillation thereof.

Among the objects of the invention are to provide a process in which carbonaceous substance deposited during the distillation and cracking of hydrocarbon oils, are treated with steam under relatively high temperatures and pressures to produce an adsorbing substance which is subsequently treated with hydrocarbon gases to produce a readily combustible fuel; to provide a process in which the deposited carbonaceous substances may be first transformed into activated carbon and then satiated with gas, producing a fuel which has a high B. t. u. content and readily combustible in any type of furnace.

With the distillation of oils such as crude oils, fuel oils, or in the pressure conversion or cracking of gas oils, fuel oils or other types of hydrocarbons which may be treated to produce refined products, there is a resultant carbonaceous substance which has the characteristic of forming in a coky mass, either suspended in the residual substance which comprises a viscous semi-solid liquid, or when treated in a coking still the carbonaceous substance may be reduced practically to dry coke. This carbonaceous material is substantially pure carbon having been deposited from the body of the oil during the conversion reaction.

Particularly in connection with the destructive distillation of hydrocarbon oils such as gas oil, fuel oil, and like hydrocarbons, there is deposited during the conversion of the oil a considerable quantity of carbon which in some instances is disposed of as waste material, and if utilized at all for fuel is difficult to burn due to its content of viscous substances which prevent efficient combustion. Also, unless treated in some manner, this deposited carbon is exceedingly oily and dirty to handle.

There is however, contained in this carbonaceous residue a considerable quantity of ingredients which may be removed and utilized for useful purposes, and at the same time converting the residue into a more desirable fuel.

To produce a fuel having a high B. t. u. content, this carbonaceous material is treated with steam at high temperatures and pressures. After being subjected to this treatment for a considerable period of time, the steam and moisture which may be present in the form of vapor, is drawn off and the material dried while being subjected to a reduced pressure. This treatment extracts the water vapor and ingredients removed by the steam treatment. After the reduced pressure treatment, the incondensable gas, or a mixture of gases suitable for heating purposes is forced under pressure into the mass of carbonaceous material. Subsequent to the steam treatment the residue is activated carbon, and when subjected to the treatment of gases under pressure, the carbon will adsorb the gases introduced thereto, giving a resultant product somewhat similar in form to petroleum coke. The treatment with incondensable gases is continued sufficiently long to secure complete adsorption of the gas by the activated carbon.

An example of the treatment is to add steam to the carbonaceous residue produced by the pressure conversion or cracking of hydrocarbon oils, and raise the temperature of the mixture from 300° to 600° F., while maintaining pressures in excess of ten pounds above atmospheric. The steam is blown through the body of the carbon in order to more thoroughly permeate and penetrate through the carbonaceous substance. This treatment is continued until the water vapors or steam has been thoroughly intermixed with the carbonaceous residue relieving from the residue certain volatile materials and objectionable ingredients to the fuel. The residue is then subjected to a reduced pressure to relieve the steam and water vapor from the carbonaceous body, after which an incondensable gas is introduced to the activated carbon and is permitted to be adsorbed into the carbon body. This incondensable gas is preferably of such a character as that formed during the cracking or destructive distillation of oils, and is normally returned and burned as fuel beneath the cracking stills. Any type of gas however, which is of a combustible character may be used, and will be readily adsorbed by the activated carbonaceous material. This gas is kept in contact with the activated carbon until the carbon body is entirely satiated, or

until complete adsorption has taken place. This adsorption action is promoted by maintaining pressure upon the gas during its contact with the activated carbonaceous material. It also causes the carbon to take up a maximum amount of gas.

Subsequent to this gas treatment, the carbonaceous body is removed from the receptacle, container or retort in which it has 10 been treated, and is ready for use as fuel.

I claim as my invention:

1. A process for making carbonaceous fuel consisting in treating the residue resulting from the destructive distillation or cracking 15 of petroleum hydro-carbons with steam under pressure, subsequently drying the

treated residue by subjecting it to a reduced pressure, and then bringing a combustible gas in contact with the material to be adsorbed thereby.

2. A process for making carbonaceous fuel consisting in treating the residue resulting from the cracking of petroleum hydro-carbons with steam under pressure, subsequently drying the treated residue by subjecting it to a reduced pressure, and in then bringing a combustible incondensable gas produced during the cracking of the hydrocarbon in contact with the material under pressure to be adsorbed thereby.

ALFRED OBERLE.